

## UNITED STATES PATENT OFFICE

WILLIAM H. LORIMER, OF CLEVELAND, OHIO

## DELUSTERED ARTIFICIAL SILK AND METHOD OF DELUSTERING

No Drawing.

Application filed January 21, 1929. Serial No. 334,127.

This invention relates to the art of delustering artificial silk or rayon and to the resulting product.

Artificial silk, unless delustered during its manufacture into threads, possesses a high sheen or luster which is in marked contrast to that of natural silk. Efforts have been made heretofore to alter this appearance so as to give the artificial silk an appearance more closely resembling natural silk. So far as I am aware such efforts have not been commercially satisfactory.

I have devised a method of delustering artificial silk, however, which gives a highly desirable product with any desired degree of luster, can be quickly, easily and inexpensively employed and possesses the additional virtue that by its use before the artificial silk is dyed, the amount of dyestuff otherwise required for a desired shade or depth of color can be materially decreased.

The present method may be practiced on artificial silk in the form of thread, hank or skein, or piece goods. It may be carried out before or during dyeing, and after dyeing in the case of certain dyes which are not dissolved or otherwise harmfully effected by the substances employed for delustering.

My invention is based on the discovery that when artificial silk or rayon is suitably brought into contact with a liquid to which has been added certain inorganic salts which react to form an extremely fine, extremely insoluble precipitate, the artificial silk or rayon is delustered in proportion to the amount of salts used, its strength and softness as present in the finished product are preserved substantially unimpaired and the delustering is permanent under the ordinary subsequent processing operations and the ordinary service conditions.

As an illustration of my invention and of substances having suitable properties I give the following detailed description:

Alum and barium chloride in the desired amounts are dissolved in hot water and added to a bath. Then the artificial silk is immersed therein under proper temperature conditions and for a length of time sufficient for the delustering action to take place. I

prefer to use approximately equal parts of the two above mentioned salts. For nearly complete delustering about one percent of each salt (based on the weight of artificial silk to be treated) has been found satisfactory but the amounts may be increased several percent with slight additional delustering. For only partial delustering the percentage of salts may be decreased so that only a small fraction of one percent of each salt is present, the degree of delustering varying with the amount of salts used.

I have found that when the delustering and dyeing are carried out in that order the amount of dyestuff required for a given shade or color can be decreased perhaps fifteen percent or more from the amount required by rayon not delustered for the same shade or color. In other words, less dye is needed when my delustering material has been used prior to dyeing to obtain a certain shade or color than when the delustering material has not been used. Conversely a different shade or color may be obtained with the same amount of dye.

The temperature of the delustering solution may vary widely, for example, from about 70° F. to about 212° F. but, since artificial silk tends to become somewhat brittle and to lose strength when heated near the boiling point of water, I prefer not to exceed about 180° F. Very good results can be obtained at temperatures from about 70° F. and about 180° F. and particularly between about 160° F. and about 180° F.

The delustering action takes place quickly where the artificial silk is in such form that the threads can be brought properly and quickly into the solution, as in the case of a single thread, and somewhat more slowly as in the case of a skein or woven piece where the skein or piece or the solution is agitated to bring about the proper contact.

The product resulting from this method has an appearance more or less resembling that of natural silk, and its strength and softness is substantially unimpaired.

When artificial silk is treated as aforesaid some action takes place, which may be due to a chemical phenomenon, by which there is

brought about such a combination between the artificial silk and certain substances in the solution that the desired delustering is accomplished.

5 Having thus described my invention in sufficient detail for those skilled in the art to understand and practice the same, what I desire to secure by Letters Patent is defined in what is claimed:

10 1. The method of delustering artificial silk which comprises providing a solution containing approximately equal parts of alum and barium chloride totalling from a fraction of one percent up to about five percent 15 by weight of the silk, and bringing the silk into suitable contact with the solution while maintaining the temperature of the solution between about 70° F. and 212° F.

20 2. The method of delustering artificial silk which comprises immersing the silk in a solution heated between about 160° F. and about 180° F. and containing approximately equal parts of alum and barium chloride totalling between a fraction of one percent and five 25 percent by weight of the silk, and bringing the silk into the solution in a manner to permit uniform delustering of the silk.

30 3. The method of delustering artificial silk which comprises providing a solution heated between about 160° F. and about 180° F. and containing approximately equal parts of alum and barium chloride totalling between about one and about three percent by weight of the silk, and bringing the silk into contact 35 therewith in a manner to permit uniform delustering of the silk.

40 4. The method of delustering artificial silk which comprises immersing the silk in a solution heated between about 70° F. and about 212° F. and containing approximately equal parts of alum and barium chloride totalling between a fraction of one percent and three percent by weight of the silk, and bringing the silk into the solution in a manner to permit uniform delustering of the silk.

45 5. The method of delustering artificial silk which comprises providing a solution heated between about 160° F. and about 180° F. and containing approximately equal parts of alum and barium chloride totalling about two percent by weight of the silk, and bringing the silk into contact therewith in a manner to permit uniform delustering of the silk.

50 6. The method of delustering artificial silk which comprises immersing the silk in a solution heated between about 70° F. and 212° F. and containing approximately equal parts of alum and barium chloride totalling about two percent by weight of the silk, and bringing the silk into the solution in a manner to permit uniform delustering of the silk.

In testimony whereof I hereunto affix my signature this 17th day of January, 1929.

WILLIAM H. LORIMER.